# EUROPEAN PATENT SPECIFICATION

(11) **EP 0 986 656 B1**
(45) Date of publication and mention of the grant of the patent: **17.11.2004**
(21) Application number: 97918786.1
(22) Date of filing: 24.04.1997
(51) Int. Cl.: D01D 5/08, A46B 1/00, A46B 9/04

(54) **MONOFILAMENTS WITH SPLIT ENDS**
MONOFILAMENTE MIT GESPALTENEN ENDEN
MONOFILAMENTS A EXTREMITES FENDUES

(43) Date of publication of application: 22.03.2000
(73) Proprietor: E.I. DUPONT DE NEMOURS AND COMPANY, Wilmington, DE 19808 (US)
(72) Inventor: RACKLEY, Robert, L., Parkersburg, WV 26104 (US)
(74) Representative: Abitz, Walter, Dr.-Ing.
(86) International application number: PCT/US1997/006780
(87) International publication number: WO 1998/048086

(56) References cited:
- EP-A- 0 450 210
- DE-A- 4 442 001
- US-A- 4 279 053
- US-A- 5 128 208

## Description

### 1. Field of the Invention

This invention relates generally to monofilaments, and more particularly to monofilaments having split ends, which may be used for example as toothbrush bristles.

### 2. Description of the Related Art

The following disclosures may be relevant to various aspects of the present invention and may be briefly summarized as follows:
US 5,128,208 to Bond *et al* discloses a synthetic polymeric paint brush bristle having the appearance and performance of natural hog bristle, having been formed from at least three strands of polymer.
US 5,953,783 to Hahn discloses a tooth cleaning apparatus that has a working surface formed by fibrous cleaning elements of different lengths and of very small diameters at their working ends. The cleaning elements are fixed on a base fabric, which is reinforced by a foam layer and thus forms a deformable hollow unit that is then attached to a handle. The pile-like cleaning elements facilitate very effective cleaning even on the fine surface contours of curved tooth surfaces.

Thermoplastic polymers have long been used to form brush bristles in a wide variety of configurations. To increase the effectiveness of these brushes, the ends of such bristles have been split or "feathered" to provide a soft bristle tip. In the past, however, various difficulties have been encountered in splitting bristle tips.

In particular, various techniques have been used to split paintbrush bristles to improve painting performance. Such procedures have been particularly suited to paintbrush bristles because long splits which propagate along a large portion (up to one inch) are particularly desirable. With certain brushes, however, only splitting of the tips is desirable. For example, the length of a typical toothbrush bristle is about (or less than) 12.4mm (one half inch). If splitting were to occur along a large portion of a toothbrush bristle, the bristles would not be sufficiently rigid to adequately clean teeth. Accordingly, cucrently available splitting techniques fail to adequately address difficulties associated with splitting the tips of toothbrush bristles and other bristles in which long splits are undesirable.

### SUMMARY OF THE INVENTION

This invention relates to a monofilament having a portion with a plurality of internal fusion lines and at least four voids, wherein the voids comprise between 5 and 20% of the cross-sectional area of the monofilament.

This invention also relates to a monofilament having a diameter in a range of 63.5 to 304.8 µm (0.0025 to 0.012 inches), wherein the monofilament has a hexalocular, an octalocular, or a near circular shape.

In addition, this invention relates to a method of manufacturing extruded monofilaments having split ends, including the steps of extruding a plurality of thermoplastic polymeric streams to form a plurality of monofilaments, spinning a plurality of cutting blades above 1000 rpm, and placing a plurality of cutting blades in contact with end portions of the monofilaments to form split ends. In one embodiment of the present invention, the blades are spun at or near the natural frequency of the monofilaments.

Accordingly, there is provided a brush monofilament as claimed in claim 1 hereinafter and a toothbrush as claimed in claim 11 hereinafter.

### BRIEF DESCRIPTION OF THE DRAWINGS

Fig. 1a is a cross-sectional view of a hexalocular monofilament of the present invention.
Fig. 1b is a cross-sectional view of a spinnerette capillary used to extrude the monofilament of Fig 1a.
Fig. 2a is a cross-sectional view of another hexalocular monofilament of the present invention.
Fig. 2b is a cross-sectional view of a spinnerette capillary used to extrude the monofilament of Fig 2a.
Fig. 3a is a cross-sectional view of another hexalocular monofilament of the present invention.
Fig. 3b is a cross-sectional view of a spinnerette capillary used to extrude the monofilament of Fig 3a.
Fig. 4a is a cross-sectional view of another hexalocular monofilament of the present invention.
Fig. 4b is a cross-sectional view of a spinnerette capillary used to extrude the monofilament of Fig 4a.
Fig. 5a is a cross-sectional view of another hexalocular monofilament of the present invention.
Fig. 5b is a cross-sectional view of a spinnerette capillary used to extrude the monofilament of Fig 5a.
Fig. 6a is a front view of a spinnerette having a plurality of spinnerette capillary locations.
Fig. 6b is a side view of the spinnerette of Fig. 6a.
Fig. 7a is a plan view of a blade used in manufacturing a monofilament having split ends.
Fig. 7b is a front view of a structure having three blades mounted on a common shaft for use in splitting the ends of the monofilaments of the present invention.
Fig. 7c is a side view of the structure of Figure 7b.
Fig. 8 is a graph of the natural frequency for a 612 monofilament with a 3792.1 KPa (550,000 psi) modulus and various lengths and diameters.
Fig. 9 is a perspective view of a toothbrush having a plurality of feathered bristles.
Fig. 10 is a side view of a plurality of bristles with split ends that produce a plurality of soft fine tips.
Fig. 11 is a side view of a comparison of a feathered toothbrush bristle which spreads-out on a tooth surface with an ordinary solid tip which provides only a single contact point.
Fig. 12 is a view of feathered toothbrush bristles which penetrate deeper at the gum line for better cleaning without hurting the gum of a patient.
Fig. 13 is a cross-sectional view of an octalocular monofilament in accordance with the present invention.

### DETAILED DESCRIPTION OF THE PREFERRED EMBODIMENTS OF THE PRESENT INVENTION

Which reference to the drawings, several embodiments of the present invention, and their corresponding method of manufacture, will now be described in greater detail. Which reference to Figs. 1a, 2a, 3a, 4a and 5a, examples of a monofilament having a hexalocular shape are shown. Such shapes were achieved through an extrusion process using the respective spinnerette capillaries of Figs. 1b, 2b, 3b, 4b and 5b. Such monofilaments were prepared by the fusion of six polymer streams. Each of these monofilaments 10 include a plurality of voids 20 and a plurality of weld or fusion lines. The voids result in a void content of between 5 and 20% of the cross-sectional area of the monofilaments.

The brush bristle of the present invention can be prepared from a wide variety of thermoplastic polymeric materials including polyamides, polyesters and polyolefins.

Polyamides for use in brush manufacturing including nylon 6,6. nylon 610 (polyhexamethylene sebaccamide), and nylon 612 (hexamethylene diamine). Polyesters which have been found particularly well suited to bristle manufacture include polybutylene terephthalate and polyethylene terephthalate. A polyolefin which has been found particularly well-suited to bristle manufacture is polypropylene.

The overall diameter, or overall maximum cross-sectional dimension, of the brush bristles of the present invention is in the range of (0.0025 to 0.012 inches) 0.064 to 0.3mm.

The bristles of the present invention are preferably formed by extruding six or more individual streams of polymeric material from a spinnerette including the spinnerette capillaries shown in Figs 1b, 2b, 3b, 4b, and 5b, and joining the streams to form a single filament. A spinnerette, such as the one shown in Figures 6a and 6b, includes a plurality of spinnerette capillaries. With reference to Figs. 1b, 2b, 3b, and 5b, in the extrusion of the thermoplastic polymer streams, the polymer is extruded through openings 40. The fusion of the streams results in fusion lines at the interface of the individual streams, and the formation of longitudinal voids along the fusion lines. The general configuration of the voids can vary widely.

After extrusion of the thermoplastic polymer streams at elevated temperatures into a single filament, the monofilament is quenched and then drawn as generally described, for example, in U.S. Pat. No. 2,418,492, herein incorporated by reference. incorporated by reference.

After extrusion and quenching of the monofilament, the filament is oriented by stretching to improve the longitudinal strength. In addition, the filament can be subjected to other treatments to improve physical properties, such as treatment with saturated steam as described in U.S. patent No. 3,595,952, herein incorporated by reference.

The filament may be heat set after drawing for good bend recovery. The heat setting can be carried out either in a gas such as by blowing hot air over the fiiament, or a liquid bath such as by passing the filament through a bath of oil. The filaments are then cut into lengths suitable for brush manufacture. The individual bristles are then gathered into bundles, the bundles are tufted into brushes, and the brushes are tipped and flagged by a procedure described below.

With reference to Fig. 7a, a plan view of a cutting blade for use in splitting the ends of the bristle of the present invention is shown. An arrangement of three such blades which are separated by spacers on a common shaft by about 4.8mm (3/16 of an inch) and which are approximately rotated from one another by 120 degrees is shown in Figs. 7b and 7c. It has been found that by rotating such a blade above 1000 rpm and placing such a blade in contact with the bristles achieves a fine feathering (splitting) effect. In one example of the present invention, the blades are rotated at 30,000 rpm with a router motor. The interference between the bristle and the blade is varied depending on the depth of the split desired, although it has been found that 3.2 to 6.4mm (1/8 to 1/4 of an inch) is preferable. Essentially by spinning the blades at a high rate of speed and placing the blades in contact with the bristle tips, a fast and violent bristle cutting action is achieved, thereby causing optimal bristle splitting.

It has also been found that by rotating the blades at or near the natural frequency of a monofilament will obtain optimal splitting of the bristles. The natural frequency of a uniform beam is$\text{Natural Frequency} \text{=} \text{A} \sqrt{\frac{\text{EI}}{{\text{ul}}^{\text{4}}}}$ where A=3.52 for a cantilever beam;$\text{I = area moment of inertia = Π} \frac{{\text{d}}^{\text{4}}}{\text{64}} \text{;}$ E is Young's Modulus of Elasticity; µ is mass per unit length; and l = length. The natural frequency is usually stated in radians per second which can also be expressed in revolutions per minute by dividing by 2π and multiplying by 60 seconds per minute.

With reference to Fig. 8, a graph of the natural frequency for a 612 monofilament bristle with a 3792.1 KPa (550,000 psi) modulus and various lengths and diameters is shown.

The monofilament bristles of the present invention produce a larger number of smaller ends ("flags") than previously known monofilament bristles of the same diameter. The bristles exhibit excellent durability and cleanability, and are particularly useful as toothbrush bristles to produce remarkably soft, fine tips. By using such a technique, the bristles of the present invention are split rather than end rounded to give a plurality of smaller ends that scrub the gingival area more effectively. It has also be found that the more dense area achieved by such flagged ends scrub major tooth areas better by keeping toothpaste in contact with the tooth surface as well as achieving a softer feel when contact is made with soft tissue in the mouth.

With reference to Fig. 9, a perspective view of a toothbrush having a plurality of feathered bristles is shown. With reference to Fig. 10, a plurality of bristles with split ends that produce a plurality of soft fine tips is also shown. These feathered filaments spread-out on tooth surfaces to provide a plurality of contact points, unlike ordinary solid tips which provide only one contact point. A comparison of these plurality of contact points to the single contact point of a solid tip is shown in Fig. 11. The fine feathered filaments of the present invention also produce a greater and deeper penetration at the gum line for better cleaning without hurting the gum line of a patient. Such deeper penetration at the gum line is shown in Fig. 12. Accordingly, these soft filament tips carry sweeping power action along with a beneficial interdental and gumline cleaning. In fact, it has been found that such feathered tips reach farther between teeth, provide better cleaning coverage than ordinary soft filament tips because of the increase in contact surfaces, and thus holds toothpaste in contact with teeth. Such an arrangement also provides a unique cushioning effect at the tips which adds extra softness to the brush. Such softness reduces bleeding of the gums during brushing. Moreover, such bristles have proven to be as hygienic as round filaments.

Although the present invention has been described with reference to a hexalocular bristle structure having six voids, it has also been found that an octalocular bristle structure (having eight voids) provides numerous beneficial effects. Such an octalocular bristle is shown in Figure 13. It is also to be understood that although six and eight streams have been used to achieve hexalocular and octalocular structures, respectively, a greater number of streams may be used to produce additional structures having a corresponding greater number of voids. The outer shape of such hexalocular, octalocular or other structures may be manufactured so as to have a circular or near circular shape. Such a near circular outer shape is shown in Figure 13.

The percentage of the cross-sectional area occupied by the voids in the monofilaments is determined by the size, location, symmetry and shape of the voids. It has been found that a certain level of hollow space (voids) will result in an optimal splitting of brushes having relatively short lengths, such as toothbrushes. The voids optimally result in a void content of between 5 and 20% of the cross-sectional area of the monofilaments. With such brushes, if the voids are too small, such as the voids disclosed in U.S. Patent No. 5,128,208, any feathering effect would result in broken bristle ends rather than in achieving feathering. If the voids are too large, such as the voids disclosed in U.S. Patent No. 4,279,053, the bristle would feather easily, but the splits would likely propagate down the bristle during use. With use as a toothbrush bristle, it is important that the tips of the bristles be split without the split propagating down the filament, either during manufacture or use by a patient. This may also be true of other types of brushes, depending on the particular use of the brush and/or length of the bristles.

With regard to the location of the voids within the monofilament, the voids should be located about 1/2 way between the center and the outside edge. It has also been found that a longer and slender void achieves a greater flagging effect than a rounded void.

It is also to be noted that the voids may be either symmetrical or asymmetrical, although it is to be noted that an asymmetrical void may have a natural curvature which is often undesirable in particular uses, such as a toothbrush. Preferably, openings 40 of the spinnerette capilaries, as shown in Figs. 1b, 2b, 3b, have a radius of curvature r in the range of 127 to 305 µm (5 to 12 mils). Openings 40 of the spinnerette capillary of Fig. 2b have an internal radius (or radius of curvature) of 229 µm (9 mils), while the openings of the spinnerette capillary of Fig. 3b have a radius of 203 µm (8 mils). Interestingly, use of the spinnerette capillary of Figure 2b results in the asymmetrical monofilament of Fig. 2a, while use of the spinnerette capillary of Fig. 3b results in the symmetrical monofilament of Fig. 3a. It is important to note that the asymmetrical monofilament of Fig. 2a is not due to problems in the symmetry of the design, but with the large size of the lobes. With large lobes, the streams are not knitted together as the center is pulled. As such, insufficient space is left for two of the streams to be pulled into the monofilament.

The void content is determined on the basis of the weight of the hollow bristle and the weight of a hypothetical solid bristle of the same exterior configuration, according to the following formula:

## Claims

1. A brush monofilament (10) having a portion with a plurality of internal fusion lines and at least four voids (20), **characterised in that** said voids occupy between 5 and 20% of a cross-sectional area of the monofilament.

2. The brush monofilament (10) of claim 1 wherein said brush monofilament (10) has a diameter in a range of 0.0064 to 0.030cm.

3. The brush monofilament (10) of claim 1 wherein said brush monofilament (10) has a near circular outer shape.

4. The brush monofilament (10) of claim 2 said monofilament (10) having a hexalocular, and octalocular, or a near circular shape.

5. The brush monofilament (10) of any preceding claim wherein said monofilament (10) is a toothbrush bristle.

6. The brush monofilament (10) of any preceding claim wherein said monofilament (10) is made of a thermoplastic polymeric materiel.

7. The brush monofilament (10) of any preceding claim wherein said thermoplastic polymeric material is selected from the group consisting of nylon 610, nylon 612, a polyamide, and polybutylene terephthalate.

8. The brush monofilament (10) of any preceding claim wherein said brush monofilament (10) has six voids.

9. The brush monofilament (10) of any of claims 1 to 7 wherein said brush monofilament (10) has eight voids.

10. A toothbrush comprising a plurality of brush monofilaments (10) of claim 1.

11. A toothbrush comprising a plurality of bristles having feathered end portions and unfeathered stem portions, **characterised in that** said unfeathered stem portions have a plurality of internal fusion lines and at least four voids (20), that said voids (20) occupy between 5 and 20% of a cross sectional area of the bristles, and that a plurality of said feathered end portions are less than 0.64 cm in length.

12. The toothbrush of claim 11 wherein said plurality of bristles are brush monofilaments (10).

13. The toothbrush of claim 11 or claim 12 wherein said plurality of bristles are made of a thermoplastic polymeric material.

14. The toothbrush of claim 13 wherein said thermoplastic polymeric material is selected from the group consisting of polyhexamethylene sebaccamide, a polyamide, and polybutylene terephthalate.

15. The toothbrush of any of claims 11 to 14 wherein each of said unfeathered stem portions have an outer diameter in a range of 0.0064 to 0.030 cm.

16. The toothbrush of any of claims 11 to 15 wherein said unfeathered stem portions have a hexalocular or an octalocular configuration.

17. The toothbrush of any of claims 11 to 16 wherein each of said feathered portions is less than 0.64 cm in length.

## Patentansprüche

1. Bürsten-Monofilament (10), das einen Abschnitt mit einer Mehrzahl von inneren Schmelzlinien und mindestens vier Hohlräumen (20) hat, **dadurch gekennzeichnet, dass** die Hohlräume zwischen 5 und 20% der Querschnittfläche des Monofilamentes einnehmen.

2. Bürsten-Monofilament (10) nach Anspruch 1, wobei das Bürsten-Monofilament (10) einen Durchmesser im Bereich von 0,0064 bis 0,030 cm hat.

3. Bürsten-Monofilament (10) nach Anspruch 1, wobei das Bürsten-Monofilament (10) eine nahezu kreisrunde äußere Kontur hat.

4. Bürsten-Monofilament (10) nach Anspruch 2, wobei das Monofilament (10) eine hexalobale und oktalobale oder eine nahezu kreisrunde Kontur hat.

5. Bürsten-Monofilament (10) nach einem der vorgenannten Ansprüche, worin das Monofilament (10) eine Zahnbürstenborste ist.

6. Bürsten-Monofilament (10) nach einem der vorgenannten Ansprüche, worin das Monofilament (10) aus einem thermoplastischen polymeren Material hergestellt ist.

7. Bürsten-Monofilament (10) nach einem der vorgenannten Ansprüche, worin das thermoplastische polymere Material ausgewählt ist aus der Gruppe, bestehend aus Nylon 610, Nylon 612, einem Polyamid und Polybutylenterephthalat.

8. Bürsten-Monofilament (10) nach einem der vorgenannten Ansprüche, worin das Monofilament (10) sechs Hohlräume hat.

9. Bürsten-Monofilament (10) nach einem der Ansprüche 1 bis 7, worin das Monofilament (10) acht Hohlräume hat.

10. Zahnbürste, aufweisend eine Mehrzahl von Bürsten-Monofilamenten (10) nach Anspruch 1.

11. Zahnbürste, aufweisend eine Mehrzahl von Borsten mit aufgefederten Endabschnitten und mit nicht aufgefederten Stengelabschnitten, **dadurch gekennzeichnet, dass** die nicht aufgefederten Stengelabschnitte eine Mehrzahl von inneren Schmelzlinien haben und mindestens vier Hohlräume derart haben, dass die Hohlräume (20) zwischen 5 und 20% der Querschnittfläche der Borsten einnehmen, und dass eine Mehrzahl der aufgefederten Endabschnitte eine Länge von weniger als 0,64 cm haben.

12. Zahnbürste nach Anspruch 11, worin die Mehrzahl der Borsten Bürsten-Monofilamente (10) sind.

13. Zahnbürste nach Anspruch 11 oder 12, worin die Mehrzahl der Borsten aus einem thermoplastischen polymeren Material erzeugt sind.

14. Zahnbürste nach Anspruch 13, worin das thermoplastische polymere Material ausgewählt ist aus der Gruppe, bestehend aus Polyhexamethylensebazinsäureamid, einem Polyamid, und Polybutylenterephthalat.

15. Zahnbürste nach einem der vorgenannten Ansprüche 11 bis 14, wobei jeder der nicht aufgefederten Stengelabschnitte einen Außendurchmesser im Bereich von 0,0064 bis 0,030 cm hat.

16. Zahnbürste nach einem der vorgenannten Ansprüche 11 bis 15, wobei jeder der nicht aufgefederten Stengelabschnitte eine hexalobale oder eine oktalobale Konfiguration hat.

17. Zahnbürste nach einem der vorgenannten Ansprüche 11 bis 16, wobei jeder der aufgefederte Abschnitte eine Länge von mindestens 0,64 cm hat.

## Revendications

1. Monofilament de brosse (10) possédant une portion avec une pluralité de lignes de fusion internes et au moins quatre vides (20), **caractérisé en ce que** lesdits vides occupent entre 5 et 20% de la surface de section transversale du monofilament.

2. Monofilament de brosse (10) suivant la revendication 1, dans lequel ledit monofilament de brosse (10) possède un diamètre dans un intervalle de 0,0064 à 0,030 cm.

3. Monofilament de brosse (10) suivant la revendication 1, dans lequel ledit monofilament de brosse (10) a une forme externe presque circulaire.

4. Monofilament de brosse (10) suivant la revendication 2, ledit monofilament (10) ayant une forme hexaloculaire et octaloculaire ou presque circulaire.

5. Monofilament de brosse (10) suivant l'une quelconque des revendications précédentes, dans lequel ledit monofilament (10) est un poil de brosse à dents.

6. Monofilament de brosse (10) suivant l'une quelconque des revendications précédentes, dans lequel ledit monofilament (10) est composé d'un matériau polymère thermoplastique.

7. Monofilament de brosse (10) suivant l'une quelconque des revendications précédentes, dans lequel ledit matériau polymère thermoplastique est choisi dans le groupe constitué de nylon 610, de nylon 612, d'un polyamide et de polybutylène téréphtalate.

8. Monofilament de brosse (10) suivant l'une quelconque des revendications précédentes, dans lequel ledit monofilament de brosse (10) possède six vides.

9. Monofilament de brosse (10) suivant l'une quelconque des revendications 1 à 7, dans lequel ledit monofilament de brosse (10) possède huit vides.

10. Brosse à dents comprenant une pluralité de monofilaments de brosse (10) suivant la revendication 1.

11. Brosse à dents comprenant un pluralité de poils possédant des portions d'extrémités ramifiées (« feathered ») et des portions de tiges non ramifiées, **caractérisée en ce que** lesdites portions de tiges non ramifiées présentent une pluralité de lignes de fusion internes et au moins quatre vides (20), **en ce que** lesdits vides (20) occupent entre 5 et 20% de la surface de section transversale des poils et **en ce qu'**une pluralité desdites portions d'extrémités ramifiées sont de moins de 0,64 cm en longueur.

12. Brosse à dents suivant la revendication 11, dans laquelle ladite pluralité de poils est composée de monofilaments de brosse (10).

13. Brosse à dents suivant la revendication 11 ou la revendication 12, dans laquelle ladite pluralité de poils est composée d'un matériau polymère thermoplastique.

14. Brosse à dents suivant la revendication 13, dans laquelle ledit matériau polymère thermoplastique est choisi dans le groupe constitué de polyhexaméthylène sébaccamide, d'un polyamide et de polybutylène téréphtalate.

15. Brosse à dents suivant l'une quelconque des revendications 11 à 14, dans laquelle chacune desdites portions de tiges non ramifiées possède un diamètre externe dans un intervalle de 0,0064 à 0,030 cm.

16. Brosse à dents suivant l'une quelconque des revendications 11 à 15, dans laquelle lesdites portions de tiges non ramifiées présentent une configuration hexaloculaire ou octaloculaire.

17. Brosse à dents suivant l'une quelconque des revendications 11 à 16, dans laquelle chacune desdites portions ramifiées est de moins de 0,64 cm en longueur.
